

# United States Patent [19]

Berwick et al.

[11] 4,284,699  
[45] Aug. 18, 1981

[54] POLYESTER BINDER COMPONENT IN  
MULTILAYER PHOTOCONDUCTIVE  
ELEMENT

[75] Inventors: Martin A. Berwick, Kendall; Edgar  
E. Riecke, Webster, both of N.Y.

[73] Assignee: Eastman Kodak Company,  
Rochester, N.Y.

[21] Appl. No.: 910,399

[22] Filed: May 30, 1978

## Related U.S. Application Data

[63] Continuation-in-part of Ser. No. 768,460, Feb. 14, 1977,  
Pat. No. 4,173,472, which is a continuation-in-part of  
Ser. No. 696,248, Jun. 15, 1976, abandoned.

[51] Int. Cl.<sup>3</sup> ..... G03G 5/05; G03G 5/10  
[52] U.S. Cl. ..... 430/96; 430/58;

430/908

[58] Field of Search ..... 96/1.5, 1.6, 908;  
430/66, 96, 58

## [56] References Cited

### U.S. PATENT DOCUMENTS

|           |         |                  |                  |
|-----------|---------|------------------|------------------|
| 3,378,370 | 4/1968  | Brancato         | ..... 430/87     |
| 3,438,773 | 4/1969  | Hayashi et al.   | ..... 430/60     |
| 3,640,708 | 2/1972  | Humphriss et al. | ..... 430/66     |
| 3,647,432 | 3/1972  | Holstead         | ..... 430/66     |
| 3,658,541 | 4/1972  | Jacoby           | ..... 430/155    |
| 3,725,329 | 4/1973  | Jacoby et al.    | ..... 260/32.8 R |
| 3,745,005 | 7/1973  | Yoerger et al.   | ..... 430/66     |
| 3,765,884 | 10/1973 | Shea             | ..... 430/66     |
| 3,775,152 | 11/1973 | Jacoby et al.    | ..... 430/155    |
| 3,865,869 | 2/1975  | Kuehn et al.     | ..... 430/66     |
| 3,932,179 | 1/1976  | Perez-Albuerne   | ..... 96/1.5     |

### FOREIGN PATENT DOCUMENTS

|         |         |                |                  |
|---------|---------|----------------|------------------|
| 792846  | 8/1968  | Canada         | ..... 260/32.8 R |
| 799555  | 11/1968 | Canada         | ..... 430/155    |
| 1356004 | 6/1974  | United Kingdom | ..... 430/155    |
| 1431415 | 4/1976  | United Kingdom | ..... 430/75     |

## OTHER PUBLICATIONS

Polyester Plasticizer for Films of Poly(N-vinyl carbazole) Xerox Disclosure Journal vol. #1, 1976, p. 31.

Primary Examiner—Roland E. Martin, Jr.

Assistant Examiner—John L. Goodrow

Attorney, Agent, or Firm—Torger N. Dahl

[57]

## ABSTRACT

A multilayer photoconductive element containing a photoconductive insulating composition and a conducting layer, such element having in association with the photoconductive composition an amorphous, water-insoluble polyester selected from the group consisting of

(a) polyesters prepared from units derived from at least one aromatic dicarboxylic acid component and at least one diol component, at least one of said acid or diol components being a non-linear monomer selected from the group consisting of an isophthalic acid component or a branched-chain alkylene diol having the formula



wherein  $\text{R}^1$  is a branched-chain alkylene group, and  
(b) polyester copolymers prepared from units derived from at least one aromatic dicarboxylic acid component and at least one diol component, at least one of said acid or said diol components being a mixture of at least two different acids or two different diols, respectively, so that a copolymer is obtained, and at least one of said acid or one of said diol components being selected from the group consisting of a non-linear monomer as defined above or a cycloaliphatic diol; with the proviso that said photoconductive insulating composition contains a minor amount of said polyester.

12 Claims, No Drawings

## POLYESTER BINDER COMPONENT IN MULTILAYER PHOTOCONDUCTIVE ELEMENT

This application is a continuation-in-part application of U.S. Patent Application Ser. No. 768,460, filed Feb. 14, 1977 now U.S. Pat. No. 4,173,472, which is a continuation-in-part application of U.S. Pat. Application Ser. No. 696,248 filed June 15, 1976, now abandoned.

### FIELD OF THE INVENTION

This invention relates in general to electrophotography and in particular to unitary multilayer electrophotographic elements which include an electrically conductive layer and a photoconductive insulating layer.

### BACKGROUND OF THE INVENTION

Electrophotographic imaging processes and techniques have been extensively described in both the patent and other literature. Generally, these processes have in common the steps of employing an electrophotographic element which is prepared to respond to imagewise exposure with electromagnetic radiation by forming a latent electrostatic charge image. A variety of subsequent operations, now well-known in the art, can then be employed to produce a record of the image.

One type of unitary photoconductive element particularly useful in electrophotography is generally produced in a multilayer structure. Such an element is prepared, for example, by coating one or more layers of an insulating photoconductive composition onto a support which previously has been overcoated with a layer of electrically conducting material. In addition, a polymeric interlayer is often interposed between the conducting material and photoconductive composition of such unitary multilayer elements to provide adhesion and/or to serve as an electrical barrier layer between the conducting material and the photoconductive composition.

Representative publications which disclose various polymeric materials which may be employed as interlayers for use in a unitary multilayer element of the type described immediately hereinabove are set forth, for example, in U.S. Pat. No. 3,640,708 issued Feb. 8, 1972; U.S. Pat. No. 3,438,773, issued Apr. 15, 1969; U.S. Pat. No. 3,745,005 issued July 10, 1973; and U.S. Pat. No. 3,932,179 issued Jan. 13, 1976.

As indicated in the above patent publications, one particularly useful component in such polymeric interlayers is a copolymer such as a terpolymer of tetrapolymer which is hydrophobic and which has a substantial number of repeating units derived from a carboxylic acid group such as itaconic acid, acrylic acid, and the like, and/or a substantial number of repeating units derived from vinylidene chloride. Although hydrophobic terpolymers and tetrapolymers prepared containing the above-described repeating units have been found to provide good adhesive properties for use in a unitary multilayer photoconductive element as described hereinabove, it has recently been determined that these hydrophobic terpolymer and tetrapolymer materials can seriously interfere with the electrical characteristics and operating properties of multilayer photoconductive layers. In particular, it has been found that the above-described polymeric materials which contain acid components, such as itaconic or acrylic acid, or units derived from a monomer such as vinylidene chloride which is subject to degradation to form

an acid (i.e., hydrochloric acid), can seriously impair the electrical characteristics of the photoconductive composition associated with said multilayer photoconductive element.

In addition to the foregoing patent publications, other patent publications such as U.S. Pat. No. 3,647,432 issued Mar. 7, 1972 and U.S. Pat. No. 3,765,884 issued Oct. 16, 1973 have described compositions composed of certain organic photoconductor or sensitizer materials admixed with any one of various binder materials. Included within the extensive listing of useful such binder materials are polycondensate polymers such as a polyester of ethylene glycol, neopentyl glycol, terephthalic acid and isophthalic acid. Although the aforementioned polyester can be employed as the binder material of a photoconductive insulating composition, it has been found that this polyester when present as the sole binder component of, for example, certain homogeneous organic photoconductive insulating compositions, can interfere with the electrical operation of the resultant photoconductive composition such that it is incapable of readily accepting an initial electrostatic charge of a magnitude within the desired operating ranges of such photoconductive compositions, i.e., 600 volts or more.

### SUMMARY OF THE INVENTION

In accord with the improved multilayer photoconductive element of the present invention wherein a photoconductive insulating composition comprising a photoconductive material admixed in an electrically insulating polymeric binder(s) is in electrical contact with an electrically conducting layer, there is provided, in association with said photoconductive composition, certain polyester materials as defined hereinbelow.

The polyester materials employed in the improved multilayer photoconductive elements of the invention are amorphous, water-insoluble polyesters selected from the group consisting of

(a) polyesters prepared from units derived from at least one aromatic dicarboxylic acid component and at least one diol component, at least one of said acid or diol components being a non-linear monomer selected from the group consisting of an isophthalic acid component or a branched-chain alkylene diol having the formula



wherein  $R^1$  is a branched-chain alkylene group, and

(b) polyester copolymers prepared from units derived from at least one aromatic dicarboxylic acid component and at least one diol component, at least one of said acid or said diol components being a mixture of at least two different acids or two different diols, respectively, so that a polyester copolymer (i.e., a copolyester) is obtained, and at least one of said acid or one of said diol components being selected from the group consisting of a non-linear monomer as defined above or a cycloaliphatic diol.

In accord with the invention, the polyester employed herein is contained in minor amounts in said photoconductive insulating composition to form together with the other polymeric binder(s) mentioned hereinabove, an optically homogeneous mixture of binders in said photoconductive insulating composition. The polyester always constitutes a minor amount of the total dry weight of all binders contained in the photoconductive insulating composition.

### DESCRIPTION OF THE PREFERRED EMBODIMENTS

The aromatic dicarboxylic acid component used to prepare the polyesters employed in the invention is isophthalic or terephthalic acid or the polyesterifiable derivatives thereof including the corresponding esters derived from said acids, for example, diethylisophthalate and dimethylterephthalate and their corresponding acid anhydrides and acid chlorides. A particularly useful dicarboxylic acid component employed in the invention is terephthalic acid and polyesterifiable derivatives thereof. If desired, the dicarboxylic acid component used in the present invention may comprise a mixture of the foregoing dicarboxylic acid materials.

Typically, the branched-chain alkylene diol component represented by structural formula I hereinabove contains a branched-chain alkylene group ( $R^1$  in formula I above) having from 2 to about 15 carbon atoms, preferably from 3 to 7 carbon atoms. Examples of suitable branched-chain alkylene groups include isoalkylene groups such as isopropylidene, and isobutylidene, branched-chain pentylene and branched-chain hexylene, though isopropylidene is preferred. The alkylene groups are attached to the diol to form symmetrical or unsymmetrical side chains. Neo-alkylene groups are generally preferred, i.e. those having at least one carbon atom connected directly with four other carbon atoms, e.g. neopentylene (2,2-dimethyl-1,3-trimethylene). Examples of suitable diols containing both types of side chains include 2,2-diethyl-1,3-propanediol; 2,2-dimethyl-1,3-propanediol (neopentyl glycol); 2-methyl-2-ethyl-1,3-propanediol; 3,3-dimethyl-1,5-pentanediol and 3,3-diethyl-1,5-pentane diol.

The term "non-linear monomer" as used in the present specification is defined to include the non-linear aromatic dicarboxylic acid isophthalic acid as well as polyesterifiable derivatives thereof and the above-described branched-chain alkylene diol materials having formula I above. These materials are included in the class (a) polyesters noted above to obtain desirable amorphous and organic solvent solubility properties in these polyesters.

In the class (b) polyesters described hereinabove the desired solubility and amorphous character are obtained by virtue of employing polyester copolymers (sometimes referred to as "copolymers" or "mixed polyesters") and by incorporating one or more non-linear monomers as defined above or a cycloaliphatic diol.

Representative cycloaliphatic diols typically have the structure



wherein  $R^2$  is a cycloaliphatic group. Suitable cycloaliphatic groups include those containing from 4 to about 12 carbon atoms, and preferably 4 to about 6 carbon atoms. Examples of suitable cycloaliphatic groups include cyclobutylene, cyclopentylene, cyclohexylene, cycloheptylene, cyclooctylene and cyclodecylene, with cyclohexylene being preferred.

It will be appreciated that, in accord with the present invention, one or more of the above-described cycloaliphatic diols may be employed, not only in the class (b) polyesters described above, but also as a diol component of the above-described class (a) polyesters.

In addition to the above-described components, the class (a) and class (b) polyesters used in the present invention may also contain any one of various straight-

chain alkylene diol materials and/or any one of various aromatic diols including bisphenols or monocyclic aromatic diols. Representative straight-chain alkylene diol components useful in preparing the polyesters employed in the present invention typically have the formula



wherein  $R^3$  represents a straight-chain alkylene group having from 1 to about 10 carbon atoms, preferably from 1 to about 4 carbon atoms. A partial listing of representative such straight-chain alkylene diols include ethylene glycol, trimethylenediol, tetramethylene glycol, pentamethylene glycol, and the like.

Representative bisphenols which may be employed are generally of the structure of formula II:



wherein each  $R^4$  and  $R^5$ , which can be the same or different, are selected from the group consisting of hydrogen atoms, aryl radicals, such as phenyl, including substituted phenyl, halogen atoms, nitro radicals, cyano radicals, alkoxy radicals and the like, and wherein the substituents on the phenyl radical may be a halogen atom, nitro radical, cyano radical; or alkoxy radical.  $R^6$  and  $R^7$  represent aliphatic, monocyclic or bicyclic radicals and can each be hydrogen atoms; alkyl radicals of from 1 to 6 carbon atoms, including substituted alkyl radicals, such as fluoromethyl, difluoromethyl, trifluoromethyl, dichlorofluoromethyl, 2-[2,3,4,5-tetrahydro-2,2-dimethyl-4-oxofur-3-yl]ethyl and the like; cycloalkyl radicals of from 4 to 6 carbon atoms, such as cyclohexyl; and aromatic radicals having from 6 to 20 carbon atoms, such as phenyl, 3,4-dichlorophenyl, 2,4-dichlorophenyl.  $R^6$  and  $R^7$  taken together with the carbon atoms to which they are attached can represent a monocyclic, bicyclic, or heterocyclic moiety having from 4 to about 10 atoms in the ring.

Typical useful bisphenols include: Bisphenol A; 2,2-bis(4-hydroxy-3,5-dichlorophenyl)propane[tetrachlorobisphenol A]; 1-phenyl-1,1-bis(4-hydroxyphenyl)ethane; 1-(3,4-dichlorophenyl)-1,1-bis(4-hydroxyphenyl)ethane; 2,2-bis(4-hydroxyphenyl)-4-[3-(2,3,4,5-tetrahydro-2,2-dimethyl-4-oxofuryl)butane]; bis(4-hydroxyphenyl)methane; 2,4-di-chlorophenyl-bis(4-hydroxyphenyl)methane; 1,1-bis(4-hydroxyphenyl)cyclohexane; 1,1,1,3,3-hexafluoro-2,2-bis(4-hydroxyphenyl)propane; diphenyl-bis(4-hydroxyphenyl)methane.

Other useful bisphenols include 1,4-naphthalenediol, 2,5-naphthalenediol, bis(4-hydroxy-2-methyl-3-propylphenyl)methane, 1,1-bis(2-ethyl-4-hydroxy-5-sec.-butylphenyl)ethane, 2,2-bis(4-hydroxyphenyl)propane, 2,2-bis(4-hydroxy-2-methyl-5-tert.-butylphenyl)propane, 1,1-bis(4-hydroxy-2-methyl-5-isoctylphenyl)isobutane, bis(2-ethyl-4-hydroxyphenyl)-4,4-di-p-tolylmethane. Still other useful bisphenols are disclosed in U.S. Pat. No. 3,030,335 and Canadian Pat. No. 576,491.

Representative monocyclic aromatic diols include hydroquinone and hydroquinones substituted with alkyl groups of 1 to about 15 carbon atoms, or halogen atoms, resorcinol, unsubstituted or substituted with lower alkyl groups or halogen atoms, and the like.

The polyesters employed in the present invention should be completely esterified so that there is little or no remaining carboxylic acid groups associated with said aromatic dicarboxylic acid component used in preparing the polyesters. One advantage of the multilayer photoconductive elements of the present invention is that these elements employ the above-described polyesters which are completely or at least substantially free of any acid functions. The presence of such acid function has been found to seriously interfere with the electrical properties of many useful photoconductive compositions, particularly organic photoconductive compositions. Although the precise reason(s) for this is not fully understood, it is believed that such acid functions can interact with, for example, organic photoconductive materials, resulting in impaired electrical performance such as electrical fatigue of the photoconductive material.

In accord with one embodiment of the invention, a preferred class (b) polyester is a copolyester which contains repeating units represented by each of the following structural formulas V, VI, and VII:



wherein Ar represents an appropriate aromatic moiety and R<sup>1</sup> and R<sup>3</sup> are as defined above.

As noted above the polyester materials employed in the present invention are amorphous, i.e., they are polymers which show no melting point transition and no definite X-ray diffraction pattern. In addition, the class (b) polyesters are random copolymers. The polyesters employed in the invention exhibit good film-forming properties and freedom from crystallinity.

Because it is desirable to employ completely esterified polyesters in the present invention, it will be appreciated that these materials are prepared using approximately equal mole amounts of the dicarboxylic acid component and alkylene glycol components. In fact, it is usual to employ a slight excess of the glycol components to assure complete esterification; or, in the alternative, to employ various purification or separation techniques subsequent to the process used for production of the desired polyester so that one can be assured of obtaining a resultant polyester which is substantially or completely esterified.

When more than one diol or more than one aromatic dicarboxylic acid component are used in preparing the polyesters employed in the invention, it will be appreciated that the specific amount of each such diol or acid may vary so long as the total amount of diol and acid components are within the above-noted range, i.e., approximately equal molar amounts of acid and diol components. The exact amount of each individual diol or acid can vary widely depending on the specific material under consideration and its properties. In general, one can readily optimize a particular combination of diol and acid components to achieve the desired polymer

properties, e.g., organic solvent soluble, film-forming, optically transparent, and etc.

In general, preferred polyesters employed in the present invention are characterized by an inherent viscosity

5 greater than about 0.4 so that optimum physical properties are obtained and by their solubility in conventional organic solvents such as chlorinated hydrocarbon solvents, for example methylene chloride, chloroform, dichloroethane, mixtures thereof and the like. As noted 10 above, the polyesters employed in the present invention are water-insoluble. Inherent viscosity of these polyesters is measured in a solution composed of a 1:1 weight ratio of phenol and chlorobenzene at 25° C. using a 0.5 weight percent polyester concentration.

15 The specific polyesters employed in the present invention represent known materials and therefore detailed discussion of various methods of their preparation are unnecessary herein. For further detail concerning their preparation, reference may be made to Example 1 20 hereby incorporated by reference: British Pat. No. 1,356,004 published June 12, 1974 and Canadian Pat. Nos. 792,846 and 799,555.

25 As set forth above, the polyesters employed in the present invention are associated with the photoconductive insulating composition of the resultant multilayer photoconductive element, as an actual component of the photoconductive composition and in a minor amount based on the total amount of polymeric binder 30 contained in said photoconductive composition. Accordingly, the polyester used in the present invention typically represents from about 1 to less than 50 percent by weight of the total amount of polymeric binder present in said photoconductive composition. In accord 35 with certain preferred embodiments of the present invention, the polyesters, when incorporated in the photoconductive insulating composition, represent from about 2 to about 20 percent by weight of the total amount of polymeric binder present in said photoconductive 40 composition. In general, the total amount of polyester component contained in a typical photoconductive composition employed in the multilayer elements of the present invention is within the range of from about 1.0 to about 40 weight percent based on the 45 total dry weight of all components of the photoconductive composition. As used herein, the term "percent by weight" represents a weight percent amount based on the dry weight of the particular composition under consideration, thus excluding any amount of liquid coating 50 vehicle which may be used in a conventional coating dope.

55 As previously mentioned, a polyester of the invention forms, together with the other polymeric binder components contained in the photoconductive insulating composition, an optically homogeneous mixture of binders. As used herein, the phrase "optically homogeneous mixture of binders" means a mixture of binders which, when viewed by the naked human eye, exhibits no greater degree of light scattering (sometimes referred to as "haze") than any one of the binders exhibits by itself. This means that a mixture of binders useful in the practice of the invention comprises polyesters and other polymeric binders that are compatible with each other, i.e., can form a solid solution with each other, thus causing no increase in light scattering. Increased light scattering is undesirable in photoconductive compositions of the invention, because such compositions provide resultant visible images which exhibit a lower

degree of resolution than they would if the degree of light scattering were less.

As suggested, the polyesters employed in the present invention have found particular utility as a minor component of organic photoconductive compositions. The incorporation of a minor amount of such a polyester into the organic photoconductive composition results in no discernible deleterious effect on the electrical operating characteristics of the resultant composition. In addition, the class (b) copolymers of the invention have been found to impart improved adhesion to organic photoconductive compositions in which they are incorporated in comparison to that exhibited by somewhat similar polyesters such as a polyester of terephthalic acid; 2,5-dichloroterephthalic acid; and ethylene glycol or a polyester of teréphthalic acid; 2,2-bis[4-( $\beta$ -hydroxyethoxy)phenyl]propane and ethylene glycol.

Suitable conducting layer materials useful in the elements of the present invention include any of a wide variety of electrical conducting supports, for example, paper (at a relative humidity above 20 percent); aluminum-paper laminates; metal foils, such as aluminum foil, zinc foil, etc.; metal plates, such as aluminum, copper, zinc, brass and galvanized plates; vacuum deposited metal layers, such as silver, nickel, chromium, aluminum and the like coated on paper or conventional photographic film base such as cellulose acetate, polystyrene, poly(ethylene-terephthalate), etc. Such conducting materials as nickel can be vacuum deposited on transparent film supports in sufficiently thin layers to allow electrophotographic layers prepared therefrom to be exposed through the transparent film support if so desired. An especially useful conducting support can be prepared by coating a support material such as poly(ethylene-terephthalate), with a conducting layer containing semiconductors dispersed in a resin. Such conducting layers both with and without electrical barrier layers are described in U.S. Pat. No. 3,245,833 by Trevoy issued Apr. 12, 1966 and Dessauer, U.S. Pat. No. 2,901,348 issued Aug. 25, 1959. Other useful conducting layers include compositions consisting essentially of an intimate mixture of at least one protective inorganic oxide and from about 30 to about 70 percent by weight of at least one conducting metal, e.g., a vacuum-deposited cermet conducting layer as described in 45 Rasch, U.S. Pat. No. 3,880,657, issued Apr. 29, 1975. Likewise, a suitable conducting coating can be prepared from the sodium salt of a carboxyester lactone of maleic anhydride and a vinylacetate polymer. Such kinds of conducting layers and methods for their preparation and use are disclosed in U.S. Pat. No. 3,007,901 by Minsk issued Nov. 7, 1961 and U.S. Pat. No. 3,262,807 by Sterman et al issued July 26, 1966. Likewise, a suitable conducting coating can be prepared from the sodium salt of a carboxyester lactone of maleic anhydride and a vinylacetate polymer. Such kinds of conducting layers and methods for their optimum preparation and use are disclosed in U.S. Pat. No. 3,007,901 by Minsk issued Nov. 7, 1961 and U.S. Pat. No. 3,262,807 by 50 Sterman et al issued July 26, 1966.

The photoconductive insulating composition employed in the multilayer elements of the present invention may be composed of a wide variety of organic, including organo-metallic, or inorganic photoconductive materials in admixture with an electrically insulating, film-forming binder material. Optically, various sensitizing materials such as spectral sensitizing dyes and chemical sensitizers may also be incorporated

therein. In general, typical photoconductive compositions employed in the present invention contain an amount of photoconductor equal to at least about 1 weight percent based on the total dry weight of the photoconductive composition and, preferably, at least about 15% by weight based on the total weight of the photoconductive composition. The upper limit in the amount of photoconductive material present in a particular photoconductive compositions can be widely varied depending upon the sensitivity of the specific photoconductor under consideration, its compatibility with a particular mixture of binders, and the like. Typically, the mixture of binders is present in the photoconductive compositions employed in the invention in an amount within the range of from about 85 to about 10% by weight based on the total dry weight of the photoconductive composition.

As indicated, a wide variety of different photoconductors, including inorganic, organic, including metallo-organic and organic polymeric photoconductors, 20 may be used in the photoconductive compositions employed in the present invention. A variety of such materials are well known in the art and an extended list thereof is considered unnecessary herein. Such materials include, for example, zinc oxide, lead oxide, selenium, various particulate organic pigment materials such as phthalocyanine pigments, and a wide variety of well-known organic compounds including metallo-organic and polymeric organic photoconductors. A 25 partial listing of representative such photoconductive materials may be found, for example, in *Research Disclosure*, Vol. 109, May 1973, page 61, in an article entitled "Electrophotographic Elements, Materials and Processes," at paragraph IV(A) thereof. This partial listing of well-known photoconductive materials is hereby incorporated by reference.

In general, the photoconductive compositions employed in the element of the present invention may be prepared in the usual manner, i.e., by blending a dispersion or solution of the photoconductive material together with a mixture of binders and coating or otherwise forming a layer of such photoconductive composition on an underlying conducting layer.

As indicated, various photoconductive compositions employed in the invention can be sensitized by the addition of amounts of sensitizing compounds effective to provide improved electrophotosensitivity. Sensitizing compounds useful in various photoconductive compositions can be selected from a wide variety of such materials, including various pyrylium dye salts such as pyrylium, bispyrylium, thiapyrylium, and selenapyrylium dye salts as disclosed in Van Allan et al U.S. Pat. No. 3,250,615; fluorenes, such as 7,12-dioxo-13-dibenzo(a,h)fluorene and the like; aromatic nitro compounds of the 55 kind described in U.S. Pat. No. 2,610,120; anthrones like those disclosed in U.S. Pat. No. 2,670,286; benzophenones, such as described in U.S. Pat. No. 2,670,287; thiazoles, such as described in U.S. Pat. No. 3,732,301; various dyes such as cyanine (including carbocyanine), 60 merocyanine, diarylmethane, thiazine, azine, oxazine, xanthene, phthalein, acridine, azo anthraquinone dyes, and the like and mixtures thereof.

Where a sensitizing compound is employed in a photoconductive composition used in the present invention, it is a normal practice to mix a suitable amount of a sensitizing compound with the coating composition so that, after thorough mixing, the sensitizing compound is uniformly distributed in the coated layer.

Other methods of incorporating a sensitizing compound or the effects thereof may, however, be employed consistent with the practice of the invention. Of course, in preparing the photoconductive compositions used in the present invention, no sensitizing is required in such layers where the particular photoconductors employed exhibit sufficient photosensitivity in the desired regions of the spectrum without use of a sensitizer. In general, although the optimum concentration in any given case will vary depending on the specific photoconductor and sensitizing compound selected, substantial speed gains can usually be obtained wherein appropriate sensitizing compound is added in a concentration within the range of from about 0.001 to about 30% by weight based on the dry weight of the photoconductive insulating composition, preferably an amount within the range of from about 0.005 to about 10% by weight based on the dry weight of the photoconductive insulating composition.

With respect to the various other binder materials which may be employed in the photosensitive compositions used in the present invention by forming an optically homogeneous mixture with the polyesters described previously, preferred binders are film-forming, hydrophobic polymeric materials having fairly high dielectric strength and good electrically insulating properties.

Typical of these materials are the following:

I. Natural resins including gelatin, cellulose ester derivatives such as alkyl esters of carboxylated cellulose, hydroxy ethyl cellulose, carboxy methyl cellulose, carboxy methyl hydroxy ethyl cellulose, etc.;

II. Vinyl resins including

a. polyvinyl esters such as vinyl acetate resin, a copolymer of vinyl acetate with an ester of vinyl alcohol and a higher aliphatic carboxylic acid such as lauric acid or stearic acid, polyvinyl stearate, a poly(vinylhaloarylate) such as poly(vinyl-m-bromobenzoate-covinyl acetate), a terpolymer of vinyl butyral with vinyl alcohol and vinyl acetate, etc.;

b. styrene polymers such as polystyrene, a nitrated polystyrene, a copolymer of styrene and monoisobutyl maleate, a copolymer of styrene and butadiene, a copolymer of dimethylitaconate and styrene, polymethylstyrene, etc.;

c. methacrylic acid ester polymers such as a poly(alkylmethacrylate), etc.;

d. polyolefins such as chlorinated polyethylene, chlorinated polypropylene, poly(isobutylene), etc.;

e. poly(vinyl acetals) such as poly(vinyl butyral), etc.; and

f. poly(vinyl alcohol);

III. Polycondensates including

a. a polyester of 1,3-disulfobenzene and 2,2-bis(4-hydroxyphenyl)propane;

b. a polyester of diphenyl-p,p'-disulphonic acid and 2,2-bis(4-hydroxyphenyl)propane;

c. a polyester of 4,4'-dicarboxyphenyl ether and 2,2-bis(4-hydroxyphenyl)propane;

d. a polyester of 2,2-bis(4-hydroxyphenyl)propane and fumaric acid;

e. a polyester of phosphoric acid and hydroquinone;

f. polycarbonates (including polythiocarbonates) such as the polycarbonate of 2,2-bis(4-hydroxyphenyl)propane;

g. polyamides;

h. ketone resins; and

- i. phenol-formaldehyde resins;
- IV. Silicone resins;
- V. Alkyd resins including styrene-alkyd resins, silicone-alkyd resins, soya-alkyd resins, etc.;
- VI. Paraffin; and
- VII. Mineral waxes.

Various coating vehicles for preparing photoconductive compositions useful in the present invention include a variety of well-known solvent materials. Typically, 10 volatile organic solvents have been found quite effective. Representative such solvents include: (1) aromatic hydrocarbons such as benzene, including substituted aromatic hydrocarbons such as toluene, xylene, mesitylene, etc.; ketones such as acetone, 2-butanone, etc.; 15 halogenated aliphatic hydrocarbons such as methylene chloride, chloroform, ethylene chloride; ethers including cyclic ethers such as tetrahydrofuran, ethylether; and mixtures of the foregoing.

In accord with one especially preferred embodiment of the present invention, the photoconductive insulating composition contained in the photoconductive element of the invention is a homogeneous organic photoconductive composition containing an electrically insulating film-forming polymeric binder and an organic photoconductor(s) in solid solution in said binder. Optionally, one or more sensitizing compounds, such as one of the above-described pyrylium, bispyrylium, thiopyrylium or selenapyrylium materials may also be incorporated therein. Such photoconductive compositions are readily coated from organic solvents and when used with appropriate sensitizing compounds exhibit very useful ranges of photosensitivity. In addition, such compositions because of their optical homogeneity provide resultant visible images which exhibit a high degree of resolution. Among the various organic photoconductive materials which may be incorporated in such homogeneous compositions are any of the various organic photoconductive materials set forth in the above-referenced *Research Disclosure* article in paragraphs IV(A)(2) through IV(A)(12). Especially useful such photoconductive materials include p-type organic photoconductors having in the molecular structure thereof one or more of the following organic groups typically referred to in the art as arylamine groups and polyarylalkane groups, respectively. Still another group of useful such p-type organic photoconductive materials useful in the photoconductive compositions employed in the present invention are various pyrrole organic photoconductors such as those described in 50 U.S. Pat. No. 3,174,854 issued March 1965 and U.S. Pat. No. 3,485,625 issued Dec. 23, 1969.

A partial listing of specific p-type arylamine-containing organic photoconductors includes diarylamines, the particular non-polymeric triphenylamines illustrated in Klufel et al, U.S. Pat. No. 3,180,730 issued Apr. 27, 1965; the triarylamines having at least one of the aryl radicals substituted by either a vinyl radical or a vinylene radical having at least one active hydrogen-containing group as described in Brantly et al. U.S. Pat. No. 3,567,450 issued Mar. 2, 1971; the triarylamines in which at least one of the aryl radicals is substituted by an active hydrogen-containing group as described in Brantly et al U.S. Pat. No. 3,658,520 issued Apr. 25, 1972; tritylamine; and various polymeric arylamine-containing photoconductors such as those described in Fox U.S. Pat. No. 3,240,597, issued Mar. 15, 1966 and Merrill et al U.S. Pat. No. 3,779,750, issued Dec. 18, 1973.

Among the various specific polyarylalkane photoconductor materials which may be used in accordance with the present invention are the polyarylalkane materials such as those described in Noe et al U.S. Pat. No. 3,274,000 issued Sept. 20, 1966; Wilson U.S. Pat. No. 3,542,547 issued Nov. 24, 1970; Seus et al U.S. Pat. No. 3,542,544 issued Nov. 24, 1970; Rule U.S. Pat. No. 3,615,402 issued Oct. 26, 1971; Rule U.S. Pat. No. 3,820,989 issued June 28, 1974; and *Research Disclosure*, Vol. 133, May 1975, pages 7-11, entitled "Photoconductive Composition and Elements Containing Same". Preferred polyarylalkane photoconductive materials useful in the present invention can be represented by the formula:



wherein D and G, which may be the same or different, represent aryl groups and J and E, which may be the same or different, represent a hydrogen atom, an alkyl group, or an aryl group, at least one of D, E and G containing an amino substituent. An especially useful polyarylalkane photoconductor which may be employed in the present invention is one having the formula noted above wherein J and E represent a hydrogen atom, an aryl group, or an alkyl group and D and G represent substituted aryl groups having as a substituent thereof a group represented by the formula:



wherein R represents an unsubstituted aryl group such as phenyl or an alkyl substituted aryl such as a tolyl group. Additional information concerning the above-described preferred polyarylalkane photoconductors can be found by reference to the foregoing U.S. Patents.

A partial listing of representative p-type photoconductors useful in the present invention is presented hereinafter as follows:

1. tri-(p-tolyl)amine;
2. bis(4-diethylamino-2-meth ylphenyl)phenylmethane;
3. bis(4-diethylaminophenyl)diphenylmethane;
4. 4-(di-p-tolylamino)-4'-[4-(di-p-tolylamino)- $\beta$ -styryl]stilbene;
5. 2,3,4,5-tetraphenylpyrrole; and
6. 1,1-bis(4-di-p-tolylaminophenyl)cyclohexane.

In accord with yet another especially useful embodiment of the present invention, the polyesters described herein may be used as an additional polymeric component of a "heterogeneous" or "aggregate" multiphase photoconductive composition as described in Light

U.S. Pat. No. 3,615,414 issued Oct. 26, 1971 and Gramza et al U.S. Pat. No. 3,615,396 issued Oct. 26, 1971. Such multiphase aggregate photoconductive compositions typically comprise a continuous binder phase containing dispersed therein a particulate, co-crystalline complex of (i) a pyrylium-type dye salt such as a 2,4,6-substituted thiapyrylium dye salt and (ii) a polymer having an alkylidene diarylene group in a recurring unit thereof, e.g., a bisphenol A polycarbonate. Preferably, although not required, one or more organic photoconductors are contained in solid solution with the continuous binder phase of the aggregate photoconductive composition. For detailed reference and other information concerning particular components and methods of preparation of the above-described aggregate photoconductive compositions reference may be made to the foregoing Light and Gramza et al patents hereby incorporated by reference.

In accord with yet a further embodiment of the present invention, the polyester materials described herein may be employed in a multilayer photoconductive element wherein the photoconductive composition is composed of two or more separate layers such as the "multi-active" photoconductive insulating composition described in copending Berwick et al application U.S. Ser. No. 639,039, filed Dec. 9, 1975, hereby incorporated by reference. Such "multi-active" photoconductive compositions contain a charge-generation layer in electrical contact with a charge-transport layer. The charge-generation layer of such a "multi-active" composition comprises an "aggregate" composition as described hereinabove, i.e., a composition having a continuous polymeric phase and dispersed in the continuous phase a co-crystalline complex of (1) a pyrylium-type dye salt such as a 2,4,6-substituted thiapyrylium dye salt, and (2) a polymer having an alkylidene diarylene group as a recurring unit. The charge-transport layer of such "multi-active" compositions comprises an organic photoconductive charge-transport material such as described in the aforementioned Berwick et al patent application, for example, a p-type organic photoconductor such as the arylamine, polyarylalkane and pyrrole materials noted earlier herein.

When the polyesters employed in the present invention are incorporated directly into the charge generation or charge transport layers of the above-described "multi-active" photoconductive elements, the amount of such polyester is typically within the range of from about 1 to about 40% by weight based on the total dry weight of the specific layer into which it is incorporated.

The following examples are presented to further illustrate the invention.

#### EXAMPLE 1

Preparation of poly(ethylene:neopentylene terephthalate 55:45)

Reaction:



-continued

+ 2CH<sub>3</sub>OH

### I. Materials and Equipment

#### A. Materials

Dimethyl terephthalate (Eastman Chemicals) 291.29 g (1.50 mole)  
 Ethylene glycol (Eastman Chemicals) 110.79 g (1.785 mole)  
 Neopentyl glycol (Eastman Chemicals) 79.67 g (0.765 mole)  
 Zinc acetate dihydrate (Allied Chemical Co.) 0.0687 g (65 ppm)  
 Antimony trioxide (J. T. Baker Chemical Co.) 0.0452 g (60 ppm)

#### B. Equipment

1000 ml two-neck round-bottom flask  
 Vigreux-claisen distillation head  
 thermometer adapter and glass tubing  
 stainless steel stirrer  
 o-ring vacuum adapter  
 short path distillation adapter and cold trap

### II. Procedure

In a 100 ml two-neck, round-bottom flask, equipped with a Vigreux distillation head and a nitrogen inlet, were placed a mixture of 291.29 g (1.50 mole) dimethyl terephthalate, 110.79 g (1.785 mole) ethylene glycol, 79.67 g (0.765 mole) neopentyl glycol, (2,2-dimethyl 1,3-propanediol) (Note 1) 0.0687 g (65 ppm) zinc acetate dihydrate, and 0.045 g (60 ppm) antimony trioxide. Before heating and throughout the prevacuum stage, nitrogen was bubbled through the mixture by means of the inlet tube which led to the bottom of the flask. The mixture was heated at 200° C. for 16 hours during which the theoretical amount of methanol was collected. The temperature was then raised to 240° C. and held there for an additional one hour. The nitrogen inlet was replaced by a stainless steel stirrer through an o-ring adapter and the Vigreux distillation head was replaced by a short path distillation adapter and cold trap through which a very carefully controlled vacuum was applied: 5 cm Hg/min to a final vacuum of 0.05 mm Hg (Note 2). The temperature was increased to 265° C. and stirring under full vacuum was continued an additional two and one-half hours, at which point the melt became so viscous that stirring was difficult. The vacuum was released with nitrogen and the polymer was allowed to cool. The product was isolated by breaking the flask.

### III. Characterization

Inherent viscosities were obtained in 1:1 (wt) phenol-chlorobenzene at 25° C. for 0.5 g/dl solutions.

Thermal transitions were obtained by differential thermal analysis at 10° C./min in nitrogen atmosphere.

Nuclear magnetic resonance spectra were obtained on a Varian T60 instrument using tetramethylsilane as an internal standard and trifluoroacetic acid as solvent. The resonance of the methyl protons of neopentyl glycol is at 1.35, the methylene protons at 4.5. The ethylene

glycol protons occur 4.9 and the terephthalate protons at 8.2. The percentage of neopentyl glycol relative to ethylene glycol was calculated from the expanded (100 Hz sweep width) and integrated spectrum of the methylene region.

Typical physical properties for the polyester were measured as follows:  
 Inherent viscosity—0.71 dl. per gm.  
 Glass transition temperature—81.5° C.  
 Percent neopentyl glycol—42.26

### IV. Notes

- 25 1. A molar ratio of 1:1.7 dimethyl terephthalate versus total glycols was used. The ratio of ethylene glycol versus neopentyl glycol was 70:30.  
 30 2. The final compositions depends markedly on the manner in which the vacuum is applied. Using the above procedure, a 0.7 excess total glycol in a 70:30 ethylene glycol versus neopentyl glycol feed ratio yields a copolymer containing about 55% ethylene moieties.

### EXAMPLES 2 AND 3

In a manner similar to that described above, a copolyester of isophthalic acid, terephthalic acid, cyclohexanedimethanol and ethylene glycol (Example 2) and a copolyester of terephthalic acid, isophthalic acid and ethylene glycol (Example 3) were prepared.

### EXAMPLE 4

Two "multi-active" aggregate photoconductor elements were prepared. Each multi-active element had a 2.0 micron thick (dry thickness) aggregate charge generation layer coated on top of a 0.4 optical density vacuum deposited nickel layer carried on a polyester film support. On top of the aggregate charge generation layer was a 14 micron (dry) thick charge transport layer. The method of preparation of the charge generation layer used in this example was similar to that described in Example 6 of U.S. Pat. No. 3,615,415 issued Oct. 26, 1971. That is, a small portion, i.e., about 270 parts by weight, of the organic solvent coating dope (described hereinbelow) used to prepare the aggregate charge generation layer was first subjected to a 2-hour period of shearing action in a Waring Blender, and then this "preblended" portion of dope was added to the remaining aggregate coating dope, the entire dope then being subjected to a brief additional period of stirring prior to coating the dope on the nickel conductive layer of the support. The organic solvent coating dope used to prepare the aggregate charge generation layer had the following composition:

|                                     |                       |
|-------------------------------------|-----------------------|
| High molecular weight polycarbonate | 27 parts<br>by weight |
| 4-(4-dimethylaminophenyl)-2,6-      | 3.9 parts             |

-continued

|                                                                   |            |
|-------------------------------------------------------------------|------------|
| diphenylthiapyrylium hexafluorophosphate                          | by weight  |
| Tritolylamine (organic photoconductive charge transport material) | 18.8 parts |
| Dichloromethane (solvent)                                         | 952 parts  |
| 1,1,2-trichloroethane (solvent)                                   | 635 parts  |
|                                                                   | by weight  |

The charge transport layer was coated from an organic solvent coating dope having the following composition:

|                                                                           |            |
|---------------------------------------------------------------------------|------------|
| Lexan® 145 polycarbonate (an intermediate molecular weight polycarbonate) | 180 parts  |
| Tritolylamine (an organic photoconductive charge transport material)      | 120 parts  |
| Chloroform (solvent)                                                      | 1700 parts |
|                                                                           | by weight  |

The only difference between the two elements was that the first element (of the present invention) contained 2.7 parts by weight of the polyester of Example 1 above in the above-described organic solvent coating dope for the aggregate charge generation layer, whereas the second element (a control) contained no such additive in the charge generation layer coating dope. The addition of the polyester additive to the charge generation layer of the element of the invention did not alter the optical homogeneity of the continuous binder phase of this layer in comparison to the control element. Upon subsequent testing, it was found that the charge generation layer of the control element exhibited significantly less adhesion to the conducting nickel layer than did the element of the present invention.

#### EXAMPLE 5

In this example a multilayer photoconductive element was prepared containing as a photoconductive composition a homogeneous organic photoconductive material containing a minor amount of the polyester material prepared as described in Example 1 above to promote adhesion of the photoconductive composition to a cellulose nitrate electrical barrier layer coated on top of a copper iodide conducting layer carried on a polyester film support. The photoconductive layer of this example had a dry thickness of approximately 7 microns and consisted of (a) 67 parts by weight of film-forming, electrically insulating polyester binder, such binder representing a polyester (outside the scope of the invention) of terephthalic acid; 2,2-bis-[ $\beta$ -hydroxyethoxy]phenyl]propane; and ethylene glycol, (b) 25 parts by weight of the organic photoconductor bis(4-diethylamino-2-methylphenyl)phenylmethane, (c) 3 parts by weight of a mixture of pyrylium sensitizing dyes, and (d) 8 parts by weight of the polyester as described in Example 1. The photoconductive layer of the resultant element was coated from dichloromethane organic solvent and, when dried, exhibited substantially improved adhesion to the cellulose nitrate barrier layer in contrast to a control photoconductive layer prepared as described above but without the above-described polyester component labelled (d). In addition, the photoconductive layer of the element which contained the polyester component exhibited excellent electrical operating properties nearly as good as the control without the

polyester (d) component, thereby indicating the polyester had no substantial adverse effect on the electrical operating properties of the element. The addition of the polyester (d) component to the photoconductive layer did not alter the optical homogeneity of this layer in comparison to the control element absent the polyester (d) component. Although the control photoconductive layer without the polyester (d) component exhibited excellent electrical properties, it exhibited poor adhesion to the underlying cellulose nitrate barrier layer in comparison to the excellent adhesion exhibited by the photoconductive layer as described above containing the polyester (d) component.

A series of additional photoconductive layers were then prepared having components (a), (b), (c) and (d) labelled above, except that the weight ratios of the (a) and (d) polyester components were varied. It was found that as the amount of the polyester (d) component began to equal and exceed the amount of the (a) component (i.e., as the polyester (d) component began to exceed more than 50% by weight of the photoconductive layer), the electrical properties of the resultant photoconductive layers deteriorated such that these layers became incapable of accepting levels of initial electrostatic charge within the normal charging range of from about 400 to 600 volts. Accordingly, as shown in this example, when the polyesters of the invention are incorporated directly into an organic photoconductive layer, it was found advantageous to use the polyester as a minor component thereof to obtain good electrical properties.

The invention has been described in detail with particular reference to certain preferred embodiments thereof, but it will be understood that variations and modifications can be effected within the spirit and scope of the invention.

What is claimed is:

1. In a multilayer photoconductive element having a photoconductive insulating composition in electrical contact with a conducting layer, the improvement wherein said element comprises, as a component of said photoconductive composition, an amorphous, water-insoluble polyester which is substantially free of any acid functions and is selected from the group consisting of

(a) polyesters having recurring units derived from at least one aromatic dicarboxylic acid component and at least one diol component, at least one of said acid or diol components being a non-linear monomer selected from the group consisting of an isophthalic acid component or a branched-chain alkylene diol having the formula



wherein  $\text{R}^1$  is a branched-chain alkylene group having from 2 to about 15 carbon atoms, and  
 (b) polyester copolymers having recurring units derived from at least one aromatic dicarboxylic acid component and at least one diol component, at least one of said acid or diol components being a mixture of at least two different acids or two different diols, respectively, so that a copolyester is obtained, and at least one of said acid or one of said diol components being selected from the group consisting of a non-linear monomer as defined above or a cycloaliphatic diol; with the provisos that (1) said photoconductive insulating composi-

tion comprises a polymeric binder(s) other than said polyester so that said polyester constitutes about 1 to less than 50 percent by weight based on the total dry weight of all binders contained in said photoconductive insulating composition and is within the range of from about 1 to about 40 weight percent based on the total dry weight of said photoconductive insulating compositions; and (2) said polyester and said other polymeric binder(s) together constitute an optically homogeneous mixture of binders.

2. In a multilayer photoconductive element having a photoconductive insulating composition in electrical contact with a conducting layer, the improvement wherein said element comprises, as a component of said photoconductive composition an amorphous, water-insoluble polyester copolymer being substantially free of all acid functions and having recurring units derived from at least one aromatic dicarboxylic acid component and at least one diol component, at least one of said acid or one of said diol components being a mixture of at least two different acids or two different diols, respectively, so that a copolyester is obtained, and at least one of said acid or one of said diol components being selected from the group consisting of a non-linear monomer or a cycloaliphatic diol, said non-linear monomer selected from the group consisting of an isophthalic acid component or a branched-chain alkyleneediol having the formula



wherein  $\text{R}^1$  is a branched-chain alkylene group having from 2 to about 15 carbon atoms; with the provisos that (1) said photoconductive insulating composition comprises a polymeric binder(s) other than said polyester so that said polyester constitutes about 1 to less than 50 percent by weight based on the total dry weight of all binders contained in said photoconductive insulating composition and is within the range of from about 1 to about 40 weight percent based on the total dry weight of said photoconductive insulating composition; and (2) said polyester and said other polymeric binder(s) together constitute an optically homogeneous mixture of binders.

3. In a multilayer photoconductive element as defined in claim 2, the improvement which comprises selecting as said amorphous, water-insoluble polyester copolymer a polyester having an inherent viscosity greater than about 0.4 and containing repeating copolyester units representing each of the following structural formulas:



wherein Ar represents an aromatic moiety,  $\text{R}^1$  represents branched-chain alkylene group having from 2 to about 15 carbon atoms and  $\text{R}^3$  represents a straight-chain alkylene group having from 1 to about 10 carbon atoms.

4. In a multilayer photoconductive element as defined in claim 2, the improvement wherein said polyester is a member selected from the group consisting of

- (a) a copolyester of terephthalic acid, ethylene glycol, and neopentyl glycol;
- (b) a copolyester of terephthalic acid, isophthalic acid, cyclohexanedimethanol, and ethylene glycol; and
- (c) a copolyester of terephthalic acid, isophthalic acid, and ethylene glycol.

5. A multilayer photoconductive element having an optically homogeneous organic photoconductive insulating composition in electrical contact with a conducting layer, said element comprising, as a component of said photoconductive composition, an amorphous, water-insoluble polyester copolymer being substantially free of any acid functions and containing repeating units represented by each of the following structural formulas:



20 wherein Ar represents an aromatic moiety,  $\text{R}^1$  represents branched-chain alkylene group having from 2 to about 15 carbon atoms and  $\text{R}^3$  represents a straight-chain alkylene group having from 1 to about 10 carbon atoms; with the proviso that said homogeneous photoconductive composition comprises a polymeric binder(s) other than said polyester so that said polyester constitutes about 1 to less than 50 percent by weight based on the total dry weight of all binders contained in said homogeneous photoconductive insulating composition and is within the range of from about 1 to 40 weight percent based on the total dry weight of said homogeneous photoconductive composition.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 990

said polyester and said other polymeric binder(s) together constitute an optically homogeneous mixture of binders.

8. A multilayer photoconductive element as defined in claim 7, wherein said polyester is a copolyester of terephthalic acid, ethylene glycol, and neopentyl glycol and has an inherent viscosity greater than about 0.4.

9. A multilayer photoconductive element having a multiphase aggregate photoconductive composition in electrical contact with a conducting layer, said element comprising, as a component of said photoconductive composition, an amorphous, water-insoluble polyester being substantially free of any acid functions and containing repeating units represented by each of the following structural formulas:



wherein Ar represents an aromatic moiety, R<sup>1</sup> represents branched-chain alkylene group having from 2 to about 15 carbon atoms and R<sup>3</sup> represents a straight-chain alkylene group having from 1 to about 10 carbon atoms, with the proviso that said aggregate photoconductive composition comprises a polymeric binder(s) other than said polyester so that said polyester constitutes about 1 to less than 50 percent by weight based on the total dry weight of all binders contained in said photoconductive composition and is within the range of from about 1 to 40 weight percent based on the total dry weight of said aggregate photoconductive composition; and (2) said polyester and said other polymeric binder(s) together constitute an optically homogeneous mixture of binders.

10. A multilayer photoconductive element as defined in claim 9, wherein said polyester is a copolyester of

terephthalic acid, ethylene glycol, and neopentyl glycol and has an inherent viscosity greater than about 0.4.

11. A multilayer photoconductive element having a multi-active photoconductive insulating composition, said composition having a charge generation layer containing an aggregate photoconductive material in electrical contact with a charge transport layer containing an organic photoconductor, in electrical contact with a conducting layer, said element comprising, as a component of said multi-active photoconductive composition, an amorphous, water-insoluble polyester copolymer being substantially free of any acid functions and containing repeating units represented by each of the following structural formulas:



wherein Ar represents an aromatic moiety, R<sup>1</sup> represents branched-chain alkylene group having from 2 to about 15 carbon atoms and R<sup>3</sup> represents a straight-chain alkylene group having from 1 to about 10 carbon atoms; with the proviso that said aggregate photoconductive composition comprises a polymeric binder(s) other than said polyester so that said polyester constitutes about 1 to less than 50 percent by weight based on the total dry weight of all binders contained in said photoconductive composition and is within the range of from about 1 to 40 weight percent based on the total dry weight of said aggregate photoconductive composition; and (2) said polyester and said other polymeric binder(s) together constitute an optically homogeneous mixture of binders.

12. A multilayer photoconductive element as defined in claim 11, wherein said polyester is a copolyester of terephthalic acid, ethylene glycol, and neopentyl glycol and has an inherent viscosity greater than about 0.4.

\* \* \* \* \*